

# UNITED STATES PATENT OFFICE.

ALEXANDRE JOSEPH MARIN, OF STOCKHOLM, SWEDEN.

## EXPLOSIVE.

1,293,154.

Specification of Letters Patent.

Patented Feb. 4, 1919.

No Drawing.

Application filed August 6, 1917. Serial No. 184,774.

To all whom it may concern:

Be it known that I, ALEXANDRE JOSEPH MARIN, a subject of the King of the Belgians, residing at Stockholm, Sweden, have 5 invented certain new and useful Improvements in Explosives, of which the following is a specification.

Since the discovery of dynamite numerous products have been successively presented as 10 being more powerful than, or, at least as equally powerful as dynamite, and sometimes as possessing superior qualities as regards stability and economy.

The most important of these products to 15 enter seriously into the front rank against dynamite was compressed guncotton; but its instability, on the one hand, and on the other the deleterious gases of its explosion, necessitating the addition of a large quantity of 20 nitrates which diminished its power, prevented its extended use in mines.

Very many explosives were also presented containing chlorates and picrates, but in 25 such a dangerous form that they threw discredit for a long time upon this kind of explosive.

Then appeared the explosives of H. Sprengel. The most powerful were liquid, acid and corrosive, very difficult for practical use. 30 Their appearance was ephemeral. Other explosives produced by the same inventor were solid some with chlorate bases and others with nitrate bases, but they could not gain any ground over dynamite owing to numerous 35 inconveniences, notably: the chlorate explosives had to be prepared upon the spot, the mixtures of the nitrate base lacked the aptness for detonation, &c. Improvements followed under the name of Favier explosives, cheddite, &c. They were supplied to 40 the miners already prepared, but they all required very strong percussion to detonate them, and their power hardly equaled that of dynamite No. 1 and was very far from 45 that of gelignite.

For a long time, hypnotized, as one might say, by the qualities of dynamite endeavors were made to produce explosives as plastic as dynamite without appreciating that this 50 plasticity, due to the liquidity of the nitro-glycerin was more an inconvenience than an advantage owing to change of state

arising from differences in temperature (congelation, exudation), and also to variations in density, which the tamping in a bore hole effects with this kind of explosive, causing partial or complete miss firing of the detonator. These inconveniences have caused plastic explosives to be excluded from the normal military supplies of the majority of 60 the larger nations. The present practice is to use explosives compressed in rigid cases not deformable under the pressure of the tamping and so to retain a uniform density.

Attempts have been made to compress explosives of ammonium nitrate, but as detonation of these explosives requires very strong detonators it is clear that the greater the compression the more numerous the miss fires. It therefore results that in practice 70 these explosives maintain a feeble specific gravity so that it is necessary to have bore holes larger than those required for dynamite. Their excessive hygroscopicity was 75 also a great inconvenience.

The progress of the electro-chemist disclosed another kind of explosive. They had for a base ammonium perchlorate mixed with combustible bodies and also explosives. Their power was superior to that of all other 80 detonating materials preconceived to the extent of explosives based on nitro-glycerin. They had nevertheless a serious disadvantage; their explosion disengaged considerable quantities of hydrochloric acid which 85 in subterranean mines rendered their employment difficult. They were also very combustible and became dangerous, if they contained materials strongly nitrated.

I had in the year 1899 remarked this great 90 defect of explosives based on ammonium perchlorate and combustible materials or explosives and had succeeded in effecting a remedy in a radical manner by the addition of an alkaline nitrate capable by its explosive 95 decomposition in the presence of a nitro-hydrocarbon of liberating a quantity of alkaline base sufficient to saturate the hydrochloric acid; but these explosives, like those of the Sprengel type of ammonium nitrate 100 had the disadvantage of being generally powderous and at feeble charging density, sometimes plastic but then very difficult to detonate even with the strongest priming.

An important improvement in this kind of explosive was to abandon forever the idea of making plastic explosives and to adopt for blasting explosives the compressed form, 5 but in this which relates particularly to the explosives with a base of perchlorate of ammonia it is necessary at once to prevent miss fire in detonation due to the compression, all of them utilizing detonators of the 10 same power as those used for dynamite, and at the same time to effect a density of charging as near as possible to that of the last explosive. The problem was arduous, it has nevertheless been practically solved.

15 It is known, as already stated, that the compression, the chief effect of which is to augment the specific gravity of the explosives, has upon the aptness for detonation of the latter an influence more marked in the 20 sense of diminution of this aptness which ends by being completely annulled. The more a blasting explosive can be compressed without destroying its aptness for detonation the more this explosive will have useful 25 power. In effect, the pressures produced by the gas of the detonation by unity of surface, augment rapidly at the same rate as the speed of detonation, proportionately as the volume occupied by the explosive decreases 30 starting from a certain limit variable with the nature of the explosive, the detonation discontinuing in spite of the use of the strongest detonators, there is no more a deflagration or combustion with slow development of pressure the explosive becoming propulsive instead of being destroyed.

35 Attempts have been made to determine by calculation the limited density of free detonation, but the result is only very approximate and even when it refers to well defined 40 chemical substances such as guncotton and nitroglycerin. When the explosive is composed of different substances mixed together more or less intimately calculation is no longer of any use, experience alone can determine the density at which one may bring by compression a given explosive, without making it lose its aptness for detonation under the action of a detonator of determined power.

With the object of discovering the degree 45 of compression to which explosives may be submitted that are based on an oxidizing mixture  $\text{NH}_4\text{ClO}_4$  plus  $\text{NaNO}_3$  and of a nitro-hydrocarbon such as the dinitro-benzene, the trinitro-naphthalene and the trinitro-toluene without destroying their aptness for detonation the usual method is adopted 50 which consists in detonating an explosive cartridge in the form of a sheet of several millimeters thick arranged on a false bottom upon a block of cast metal perforated through and through. The only modification used consists in effecting the detonation

of the cartridge in contact with the sheet, 55 not directly with the detonator, but by the intermediary of another cartridge of the same explosive brought by compression to the same density and primed with a detonator of a chosen power. The primed detonator was placed in contact end to end with the cartridge touching the sheet. The one was separated from the other by a space of several centimeters. It is understood that the cartridges used were provided with their 70 envelopes of paraffin paper so that, even when they were in contact they were separated by the thickness of their envelopes. The detonation of the primed cartridges was considered as free, when it communicated the 75 detonation to the second cartridge with a neatness sufficient for the latter to perforate the sheet like a punch.

*Composition of explosives tested.*

|                                                                                         | M 2N—B | M 3N—T | 85 |
|-----------------------------------------------------------------------------------------|--------|--------|----|
| Mixture formed of 47 parts of $\text{NH}_4\text{ClO}_4$ and 34 parts of $\text{NaNO}_3$ |        |        |    |
| $\text{NO}_3$ -----                                                                     | 71     | 66     | 90 |
| Dinitro-benzin-----                                                                     | 29     | —      | 34 |
| Trinitro-toluene -----                                                                  | —      | —      | —  |
|                                                                                         | 100    | 100    |    |

In order to simplify the description and 95 to render it clear these explosives will be hereinafter designated by their initials.

By compression these explosives were successively brought to specific gravities varying from 1.2 or 1.6 and tested as regards 100 their aptness for detonation under these different densities. One is compelled only to use for these experiments detonators No. 6 similar to those used for dynamite in order that the advantages resulting from the 105 augmentation of the specific gravities of the explosive may not be compensated by the obligation to use a more powerful detonator.

In order to avoid very dangerous explosive powders and to facilitate the compression the explosive mixtures M.2N—B and M.3N—T are prepared by the wet method. The quantity of water added varies with the power of absorption of water of the explosive mixtures. The mixtures M.2N—B and M.3N—T may only contain 2 to 5 per cent. since difficulties are encountered during the desiccation in the form of crystalline efflorescence on the surface of the compressed 115 cartridges.

The results were as follows:—

M.2N—B, tested under three different densities: 1.2; 1.25 and 1.3. At the density of 1.3 the detonation was still effected at the 125 unprimed cartridge, but only if the cartridges were in contact.

M.3N—T, tested at densities varying be-

tween 1.45 and 1.6, at the density of 1.6 the unprimed cartridge still detonated if the two cartridges were in contact.

With M 3N-T compressed up to a density of 1.5 the detonation was reproduced from one cartridge to another even when separated by a space of 20 m.m.

Theory indicates for the explosives M 2N-B and M 3N-T limited densities for free detonation in the neighborhood of 1.46. The experimental results are in complete contradiction to those given.

It is to be inferred from these tests that the limited density for free detonation was in practice limited to a density of about 1.3 for the explosive M 2N-B, and about 1.6 for M 3N-T.

These results acquired and checked by repeated experiments have been put to the proof in the same conditions with mixtures formed from equal parts of the explosives previously tested, viz:

Explosive M.B.T. formed from equal parts of M.2N-B and M.3N-T.

With the explosive compressed to a density of 1.3 detonation occurred at the unprimed cartridge even with a space of 20 m.m. between the cartridges. Compressed to a density of 1.4 no detonation of the unprimed cartridge was obtained with an interval between the cartridges but the detonation was transmitted when the cartridges were in contact.

In conclusion it may be said that, by the mixture of the explosives studied, explosive products are obtained which by compression, lose their aptitude for detonation more rapidly than their components.

The relation between the specific gravity which can be given practically by compression to explosives having a base of oxidizing mixture,  $\text{NH}_4\text{ClO}_4$  and  $\text{NaNO}_3$  without destroying their aptitude for detonation, and the nature of either of the nitro-hydrocarbons which enter into their composition, have never been studied hitherto, in spite of the importance which the question presents of the charging density of blasting explosives recommended to replace dynamite.

The explosive M.3N-T has been submitted to special experiments with the object of ascertaining if the increase in the density by compression augments its sensitiveness to mechanical shocks and consequently the danger resulting from its manipulation or from its manufacture. It has occurred to the inventor that the shock of the cased bullets of modern military rifles, fired at a short range against an iron plate sufficiently thick to arrest nearly every shot, may be considered as equal to the most intense shock likely to occur in practice. The explosive cartridges studied brought by compression to the density at which they can yet detonate freely

with detonator No. 6 were inclosed in tin tubes and placed against an iron plate about 10 m.m. thick. The distance between the muzzle of the rifle and the cartridge was about 12 meters. In these conditions the explosive M.3N-T in a pulverulent state detonated freely under the shock of the bullet. Whereas when it was compressed to a specific gravity of 1.5 it did not detonate. It has been concluded from the experiments that as regards safety or stability the increase in density obtained by compression had a favorable influence on the explosives in question. The explosive M.3N-T, was tested as regards its power in an Abel lead cylinder modified according to the views of the 5th Congress of Applied Chemistry. By this means there was an enlargement of 437 c.m.<sup>3</sup>.

The more important explosives with a base of chlorate and of ammonium nitrate which alone have gained ground over dynamite, such as cheddite and Favier explosive or ammonite have also been tested in lead cylinders of the same type, producing:—

Cheddite  $\text{NO}_3$ , an enlargement of 285 c.m.<sup>3</sup>

Favier explosive No. 1 an enlargement of 295 c.m.<sup>3</sup>

Nobel's dynamite No. 1 gave an enlargement of 300 c.m.<sup>3</sup> and gelignite 432 c.m.<sup>3</sup>

Of all the explosives presented as capable of supplanting dynamite in mine work, the explosive M.3N-T is one of the most powerful. There is thus established a most serious advance over all the endeavors to replace explosives based on nitro-glycerin and guncotton by more stable products.

In addition to the explosive mixtures above mentioned and which constitute in their composition two nitro-hydrocarbons of different origin, I have studied, as regards the effect of compression on their aptitude for detonation, several other mixtures based on oxidizing salts  $\text{NH}_4\text{ClO}_4 + \text{NaNO}_3$ , additions of a mixture of different nitrated derivatives of the same hydrocarbon, such as the trinitro and tetrinitro-naphthalene.

I claim:—

1. A process for producing compressed solid safety explosives detonating freely in the open air with a No. 6 detonator, consisting in mixing ammonium perchlorate, sodium nitrate, and a nitro-hydrocarbon with a small quantity of water and compressing the mixture so as to give it a density of 1.25 to 1.6 after drying, substantially as hereinbefore set forth.

2. A process for producing compressed safety explosives detonating freely in the open air under the explosive shock of a No. 6 detonator, consisting in mixing 66 parts by weight of a mixture formed of 47 parts by weight of ammonium perchlorate and of 34

parts by weight of sodium nitrate, with 34 parts by weight of trinitro-toluene, the substance being mixed after being humidified with 2 to 5 per cent. of water and compressed into any suitable form in such a manner that the specific gravity of the explosive is between 1.45 and 1.6 and does not exceed this degree after desiccation.

In testimony whereof I have signed my name to this specification in the presence of 10 two subscribing witnesses.

ALEXANDRE JOSEPH MARIN.

Witnesses:

H. W. HARRIS,  
JACOB BAGGE.